

## UNITED STATES PATENT OFFICE

2,602,018

MONOMETHYLOL DIMETHYL HYDANTOIN  
AND DIMETHYLOL UREA TO SHRINK-  
PROOF AND CREASEPROOF CELLULOSE  
FABRICS

Leo Beer, Montreal, Quebec, Canada

No Drawing. Application January 3, 1950, Serial  
No. 136,661. In Canada December 22, 1949

2 Claims. (Cl. 8—116.3)

1

## INTRODUCTION

This invention relates to a process of imparting to cellulosic textile fabrics crease-resistance of improved permanence against washing combined with permanent boil-fast shrink-proofness. This application is a continuation-in-part of application S. N. 130,609 filed December 1, 1949.

This process is applicable to textile fabrics selected from the group consisting of natural cellulose, regenerated cellulose, mixtures of a plurality of the foregoing types in any proportion, and mixtures of one or more of the said types with up to about 50% of a cellulose ester of an organic acid, for example, cellulose acetate.

## PRIOR ART

Fabrics made from these cellulosic materials not only have the tendency to shrink in washing but also to deteriorate rapidly in appearance and to lose their freshness when crushed, twisted, or otherwise subjected to localized physical force. Therefore, these fabrics are often subjected to processes attempting to render them crease-proof so as to maintain their freshness in appearance. For crease-proofing, the textile materials are generally treated with watery solutions of ureaformaldehyde or melamine-formaldehyde precondensates under specific conditions. If such processes are carried out under tensionless working conditions, it might sometimes be expected that the treated material would in addition to being crease-proofed, be stabilized against shrinkage when washed.

For example, according to U. S. Patent 2,088,227 Tootal Broadhurst Lee Co., a resin precondensate is prepared having a mol ratio of 1:1.6 of urea to formaldehyde. The patent states that such solutions consist mainly of a monomethylol urea or mixtures thereof with dimethylol urea. The aqueous solutions of monomethylol urea or mixtures of monomethylol urea and dimethylol urea are very sensitive to acid conditions. By adding a dilute mineral acid or even by adding a solution of a weak organic acid as for example, acetic acid, to a watery solution of monomethylol urea or mixtures of monomethylol urea with dimethylol urea, a flocculent amorphous precipitate will be formed almost instantly, whereas dimethylol urea in aqueous solution will give a white amorphous precipitate only on standing for several hours if dilute mineral or organic acids are added. Therefore, the patentees assert that in such solutions it is found that free acid and particularly strong acid causes precipitation of a further condensation product whereas if the acid is replaced

by the corresponding ammonium salt a relative stability of the solution is obtained. The patent warns that the impregnating solution must not be too fully condensed, otherwise the molecular weight of the partial condensate will be so large that it cannot penetrate within the fibres. Claim 2 of this U. S. patent reads:

Process of improving the crease resistance of textile materials which consists in impregnating the material with a solution of a partially condensed resin components which is unstable in acid solution and which solution contains a potentially acid ammonium salt and heating the impregnated material to insolubilize the resin and produce a crease resisting product.

According to these patents, the treating solution has to be acidified with an organic acid to a pH of 4.5 or, for instance, if diammonium phosphate or another potentially acid substance of the amino type is used as a catalyst, the acidity of the impregnated, dried textile material should also show a pH of 4.5.

But, the crease-proof effect or the reduced tendency towards shrinkage achieved by the method of the patent is only effective for a limited time if the goods are washed at elevated temperatures in aqueous soap solution. This is because the resin formed within the fibres by repeated washing operations leaches out, and both the crease-proofing effect and the initial stabilizing effect is continuously diminished by these successive washings. This is a serious defect of which users of the process have always complained. In addition, a comparatively high concentration of the formed urea formaldehyde resin is necessary to produce a satisfactory anti-crease effect. As a general rule from about 12 to about 15% resin based on the weight of the dry fabric treated has to be formed within the fibers to achieve the desired effect. But, in all cases, due to the high resin concentration necessary to produce the desired anti-crease effect it is a very well-known fact that rayon fabrics treated for this purpose have a highly diminished resistance to abrasion compared with untreated material. The loss amounts in the average, to about 30%.

In co-pending application Serial Number 130,609 filed December 1, 1949, the applicant has disclosed the use, in shrinkage control of textile fabrics, of an aldehyde donor compound which is soluble in water and is capable of splitting off aldehyde under both acid and alkaline conditions. Such a compound selected from the group consisting of monomethylol dimethyl hydantoin and dimethyl hydantoin formaldehyde is capable of forming with the fibres, under acid conditions,

linkages which are stable to hydrolysis and characterized by a reduced swelling capacity when soaked in water or aqueous soap solutions. The aldehyde donor used in accordance with the present invention is monomethylol dimethyl hydantoin.

The applicant has now found that this type of shrinkage control can be successfully combined with crease-proofing. The treated fabric exhibits no loss of wearing qualities and practically no loss of abrasion resistance. This is done in accordance with the present invention by subjecting the textile fabric to the action of a solution containing the aldehyde donor compound, and also a dimethylol urea precondensate made from urea and formaldehyde in a molar ratio from 1 urea to at least 2 formaldehyde. The solution contains a selected non-volatile organic or inorganic acid to obtain a pH from about 2 to about 2.5. Because of this combined treatment with the aldehyde donor of the type described and dimethylol urea, in most cases comparatively small amounts only of the latter, for example, from about 3 to about 10% on the weight of the fabric (100% pick-up) need be employed to achieve satisfactory crease-proofing. The amounts of dimethylol urea will vary with the construction of the fabric. The fact that such low amounts can be used effectively apparently flows from the reduced swelling capacity of the fibre resulting from the action of the aldehyde donor. The above amounts will, of course, vary as the pick-up departs from 100% which is the preferred condition.

Broadly speaking, the process of the present invention employs the aqueous solution of the aldehyde donor which solution is nearly neutral and dimethylol urea and contains a water-soluble non-volatile organic or inorganic acid or a mixture of organic and inorganic acids, a catalyst, capable of giving the solution a pH from about 2 to about 2.5. Suitable organic acids are, for example, oxalic acid, lactic acid, citric acid, tartaric acid, and other non-volatile organic acids or mixtures thereof strong enough to catalyze the reaction. Suitable inorganic acids are, for example, boric acid and phosphoric acid. According to the invention, textile materials of the type described are thoroughly wetted i. e. impregnated with the solution containing the aldehyde donor, dimethylol urea, and the acid catalyst. The solution may or may not contain a wetting agent. The solution may or may not contain a small amount of sodium sulphate, as for example, taught in co-pending application S. N. 130,609. The solutions described are satisfactorily stable for a period of time for practical application according to the invention. The surplus of the impregnating liquor is mechanically removed, for instance by squeezing or other means allowing a pick-up of a predetermined percentage, for example a 100% liquid retention on the basis of the dry weight of the goods. They are then tensionless dried preferably at 200° F. to 240° F. and finally cured or baked from about 2 to about 5 minutes at 212° F. or higher. After curing, the fabrics are neutralized with an alkali, for example, soda ash, eventually soaped, rinsed, hydroextracted and dried without tension before putting into industrial channels of trade or before making the physical measurements referred to in the comparative tests below.

In the aqueous impregnating solution, the suggested range of concentration of the monomethylol dimethyl hydantoin is from about 1%

to about 7.5% (preferably from about 1 to about 5%) based upon the weight of the treating solution. The amount of the stabilizing compound or compounds employed should be equivalent to an amount effective to furnish from about .2% to about 1.5% (preferably from about .2% to about 1.0%) of active available formaldehyde based on the weight of the aqueous solution (at 100% pick-up based on the dry weight of the goods) and in addition a certain amount of dimethylol urea, depending on the construction of the woven or knitted textile material to be treated.

Fabrics of viscose rayon or cuprammonium yarns so processed are further improved as borne out by the fact that they show less tendency to fuzz during washing as compared to an untreated material similarly washed.

It should also be explained that if solutions containing monomethylol urea or mixtures of this compound with dimethylol urea are mixed with a solution, plus an acid catalyst effective to give a pH from about 2 to about 2.5, polymerization takes place within the solution almost immediately. Unexpectedly, however, if the monomethylol urea or mixtures of monomethylol urea with dimethylol urea are replaced in the solutions by dimethylol urea alone, the solutions are sufficiently stable for a suitable period of time to allow their technical application and if at the same time the amount of dimethylol urea is sufficient they will impart the desired crease-proofing effect.

Treated with the solution of an aldehyde donor of the type described and the necessary amount of dimethylol urea, the crease-proof effect is excellent and remains nearly unchanged after several washings even at the boil. Especially good results are achieved using lactic acid or a mixture of lactic and oxalic acids as the catalyst. The hand of the treated material is soft and no discoloration is evident from the treatment.

As a result of the process, the treated fabrics show in addition to the permanent boil-fast shrink-proofing effect of my prior application Serial Number 130,609, excellent crease-proofing characteristics notwithstanding repeated washing at temperatures even up to the boiling point.

Before treatment all traces of starch, gums, glue or natural resins and other sizing agents should first be removed from the fabric in order to permit the aqueous treating solution to penetrate the fibrous material and enter the heart of the fibres.

If desired, the "hand" or body of the goods treated can be modified in the direction of either softness or a stiffer finish at will by the introduction to the impregnating baths of suitable agents such as cation softeners for the former effect or such vegetable or animal colloids as starches, gums, glues, gelatin, modified starches, or solutions or dispersions of polyvinyl alcohol, etc. for the latter effect.

This invention will more clearly be understood by reference to the following examples. It is to be understood, however, that these examples are merely illustrative of the process and that the invention is not limited thereto, but rather is defined in the appended claims. In the examples, the term "check" has the meaning of untreated or original material.

#### EXAMPLE

Swatches of a spun viscose rayon fabric were treated for the purpose of obtaining crease-proof-

ing combined with shrink-proofing by treating with aqueous solutions of the following compositions. The "check" was not treated.

|                                                  | 1  | 2   | 3  | 4  |
|--------------------------------------------------|----|-----|----|----|
| Monomethylol dimethyl hydantoin, g.              | 20 | 30  | 30 | 25 |
| Dimethylol urea 100%, g.                         | 40 | 40  | 60 | 80 |
| Oxalic Acid, g.                                  | 6  |     |    | 3  |
| Lactic Acid 50%, g.                              |    | 120 | 70 | 60 |
| Na <sub>2</sub> SO <sub>4</sub> Anhydrous, g.    | 4  | 4   | 4  | 4  |
| "Igepal CTA Extra" (Wetting agent non-ionic), g. | 1  | 1   | 1  | 1  |
| Water to make.                                   | 11 | 11  | 11 | 11 |

The respective swatches were immersed in the above solutions afterward they were squeezed to 100% liquor retention. They were then dried without tension at 180° F. and baked for 3 minutes at 300 to 310° F.

They were neutralized then with soda ash, washed, rinsed, hydro-extracted and dried without tension. To measure their shrinkage in washing they were laundered together with the untreated check sample by the accelerated 1 hour wash test described in U. S. A. Federal specification CCC-T-191A Cotton Wash Test.

Other samples were subjected to tensile strength and abrasion resistance measurement.

#### Warp Shrinkage and Percentages

| Sample Identification | Scoured | 1 hour wash test |       |       |                 |
|-----------------------|---------|------------------|-------|-------|-----------------|
|                       |         | 1st              | 2nd   | 3rd   | Total Shrinkage |
| Check.....            | -8      | -9.5             | -10.8 | -12.7 | 12.7            |
| #1.....               | -7.5    | 0                | -0.28 | -0.3  | 7.8             |
| #2.....               | -7.2    | 0                | 0     | 0     | 7.2             |
| #3.....               | -7.8    | -1.2             | -1.2  | -1.3  | 9.1             |
| #4.....               | -7.0    | +0.2             | +0.4  | +0.3  | 6.7             |

A. WARP TENSILE STRENGTH (LBS. GRAB TEST)  
B. ABRASION (TABER CYCLES)

|            | A.  | B.  |
|------------|-----|-----|
| Check..... | 56  | 300 |
| #1.....    | 56  | 250 |
| #2.....    | 55½ | 350 |
| #3.....    | 56  | 320 |
| #4.....    | 55  | 280 |

The treated samples had a full soft hand and a very satisfactory degree of crease-proofing was obtained which practically appeared undiminished after 3 wash tests at the boil. The achieved stabilization is good as can be seen from the above figures, with practically no change in tensile strength or abrasion resistance. Very good crease-proof effect was achieved with high per-

manency. No discoloration had taken place due to the treatment.

I claim:

1. A process of imparting improved crease-resistance against washing and boil-fast shrinkage control of a cellulosic textile fabric selected from the group consisting of natural cellulose, regenerated cellulose and their mixtures with up to 50% of cellulose acetate, the steps of impregnating said fabric with an aqueous solution of monomethylol dimethyl hydantoin, said aldehyde donor being present in a concentration ranging from 1 to 7% by weight of the aqueous solution which, upon baking, decomposes to form from 0.2 to 1.5% of available active formaldehyde and from about 3 to 10% by weight of the fabric of dimethylol urea comprising 1 mol of urea and 2 mols of formaldehyde, and a water-soluble non-volatile acid in a concentration such as to give to the solution a pH of from about 2 to about 2.5, removing the surplus liquid from the material, drying the material at a temperature of from 180° to 240° F., baking the dried fabric at a temperature of from 212° to 310° F. for a time sufficient to effect reaction between liberated formaldehyde and the textile fabric, and neutralizing and washing the fabric to remove acid and reaction byproducts thereby to provide a fabric which is crease-resistant and shrinkage-controlled and which has substantially retained its original tensile strength and color.
2. The process of claim 1, wherein the acid is selected from the group consisting of oxalic acid, lactic acid, citric acid, tartaric acid, boric acid, and phosphoric acid.

LEO BEER.

#### REFERENCES CITED

The following references are of record in the file of this patent:

#### UNITED STATES PATENTS

| Number       | Name            | Date          |
|--------------|-----------------|---------------|
| 2,108,520    | Wolf et al.     | Feb. 15, 1938 |
| 45 2,159,743 | Latham et al.   | May 23, 1939  |
| 2,347,024    | Beer            | Apr. 18, 1944 |
| 2,412,832    | Pfeffer et al.  | Dec. 17, 1946 |
| 2,441,859    | Weisberg et al. | May 18, 1948  |

#### FOREIGN PATENTS

| Number  | Country       | Date           |
|---------|---------------|----------------|
| 547,846 | Great Britain | Sept. 15, 1942 |
| 880,185 | France        | Dec. 18, 1942  |

#### OTHER REFERENCES

Chemical and Engineering News, Nov. 3, 1947, page 3243, and Feb. 9, 1948, page 415.